

## UNITED STATES PATENT OFFICE

2,172,465

## INK FOR TRANSPARENT PROJECTION STRIPS

Millard Demarest, Hackensack, and Kirtland Flynn, East Orange, N. J., assignors to Celluloid Corporation, a corporation of New Jersey

No Drawing. Application November 20, 1931,  
Serial No. 576,426

## 4 Claims. (Cl. 134—35)

This invention relates to transparent strips having characters printed thereon, which strips may be employed to project desired information by means of light upon a screen.

5 An object of our invention is to prepare strips made of organic derivatives of cellulose for light projection purposes which have superior properties to strips heretofore employed. A further object of our invention is to prepare an ink which 10 is eminently suitable for the printing of characters on strips of organic derivatives of cellulose as well as the strips made of other material heretofore used for projection purposes. Further objects of our invention will appear from the following detailed description.

More or less transparent strips or ticker tape having stock market quotations or other information printed thereon have been employed in light projection machines to project such quotations upon a screen. Highly calendered paper known as glassine or foils of reconstituted cellulose have been used for this purpose, but they have not been wholly satisfactory due to the physical or chemical properties of these materials.

25 We have found that strips made of thin foils of cellulose acetate or other organic derivative of cellulose have properties which are vastly superior to those of the materials heretofore employed for making stock quotation tapes that are 30 to be employed in light projection purposes. Among the advantages of the use of cellulose acetate or other organic derivative of cellulose foil over reconstituted cellulose foil or glassine, the following are cited.

35 Foils made of cellulose acetate or other organic derivatives of cellulose have a much higher transparency than that of foils made of reconstituted cellulose so that a clearer and sharper projection, free from streaks, is obtained on the screen.

40 Foils of cellulose acetate or other organic derivatives of cellulose are materially less affected by changes in atmospheric conditions such as humidity, temperature, etc. than reconstituted cellulose. Whereas strips made of reconstituted cellulose

45 produce buckling, shrinking and distortion troubles with fluctuations in room temperatures or humidity, these phenomena do not occur with foil made of cellulose acetate or other organic derivatives of cellulose. Since reconstituted cellulose foil tends to absorb a large proportion of moisture, it tends to swell and thus bind in the projection machines where the clearance is small, and furthermore in damp weather such reconstituted cellulose foil absorbs so much moisture 50 that the layers thereof in the roll stick together

rather firmly and thus interfere with unwinding. Foils of cellulose acetate do not have these drawbacks.

Foils of cellulose acetate, being thermoplastic and soluble in certain organic liquids, may be 5 readily cemented together with solvents such as diacetone alcohol, triacetin, etc. or by heat to form neat joints or splices. Foils of reconstituted cellulose, on the other hand, are not thermoplastic and are not soluble in the usual solvents, 10 and therefore the splices of joints of reconstituted cellulose strips are awkward in appearance and are so bulky as to interfere with the proper feeding in the projection machines.

Foils made of cellulose acetate or other organic derivatives of cellulose, particularly when they contain triphenyl phosphate or other fire retardants, are less inflammable than reconstituted cellulose or paper, and this is a very important consideration in projection machines, where high 20 temperatures due to the powerful light source prevail.

In the use of projection strips, ink is applied thereto with rubber or other type wetted by means of a felt wheel to which ink is applied once a day. The printed strip or foil is immediately passed 25 mechanically before a light which projects the characters upon a screen. The ink need not necessarily be dry before projection, and the strip or foil is rolled upon the other end of the machine. If the strip is made of paper or reconstituted cellulose, the roll, smeared with ink, cannot be 30 reclaimed and must be discarded. On the other hand, in the case of foils made of cellulose acetate or other organic derivatives of cellulose, the 35 ink may be washed or bleached away and the foil reused, or the foil may be redissolved in solvents and new foil cast from the resulting solution.

Due to the superior strength of cellulose acetate foil, the cellulose acetate foil employed in 40 this invention may be thinner than is required of reconstituted cellulose foil, whereby a great saving in cost is effected.

It will therefore be seen that foils of cellulose acetate are much superior to other foils or paper 45 for use as projection strips.

However, we have found that the ordinary ink used in stock quotation recording machines, which consists essentially of a mixture of Methyl Violet and Methylene Blue dissolved or dispersed 50 in glycerine to which alcohol is added, is not absorbed smoothly and uniformly by cellulose acetate foils and therefore do not produce satisfactory markings thereon. After a long investigation, we have discovered that an ink or marking 55

fluid made of a dye or pigment dispersed or dissolved in a liquid that is a solvent plasticizer for the cellulose acetate or other organic derivative of cellulose, is eminently suitable for marking not only cellulose acetate foil, but also for marking reconstituted cellulose, paper and other material.

The thin foil employed in accordance with our invention preferably is made of an acetone-soluble cellulose acetate, but it may be made of other suitable cellulose acetates or other organic derivatives such as cellulose formate, cellulose propionate and cellulose butyrate, ethyl cellulose, methyl cellulose and benzyl cellulose. Besides the organic derivative of cellulose, the foil preferably contains plasticizers for the organic derivative of cellulose, in amounts say of 20 to 50% of the weight of the derivative of cellulose present, at least part of which plasticizer is preferably a fire retardant such as triphenyl phosphate. Examples of plasticizers for cellulose acetate are diethyl phthalate, dimethyl phthalate, triacetin, a mixture of ortho- and para-ethyl toluene sulfonamid, diethyl tartrate, dibutyl tartrate, etc.

By way of example, the following composition of a foil that may be used in accordance with this invention is given.

|                                      | Parts by weight |
|--------------------------------------|-----------------|
| 30 Acetone-soluble cellulose acetate | 100             |
| Triphenyl phosphate                  | 15              |
| Diethyl phthalate                    | 15              |

To show the superior properties of such cellulose acetate foils over reconstituted cellulose foil and the transparent paper known as glassine, the following table of physical properties is given.

|                              | Elongation | Water absorption in saturated air |         | Permeability in grams of water per square foot per 24 hrs. at 20 mm. pressure |
|------------------------------|------------|-----------------------------------|---------|-------------------------------------------------------------------------------|
|                              |            | Percent                           | Percent |                                                                               |
| 40                           |            |                                   |         |                                                                               |
| 45 Cellulose acetate foil    | 20.7       | 4.7                               | 32.7    |                                                                               |
| Reconstituted cellulose foil | 9.7        | 38                                | 50.6    |                                                                               |
| Glassine                     | 0.7        | 17.1                              | 36.2    |                                                                               |

The cellulose acetate foil used as projection strips in accordance with this invention may be of suitable thickness, say on the order of 0.001".

The strips of cellulose acetate foil that may be used for projecting may be of any suitable width in accordance with the desired purpose.

Such strips may have the width of ordinary stock quotation ticker tape, or they may be considerably wider whereby news or other information may be printed thereon to be projected on a screen. When used in newspaper sheet form,

the ink on the strip is preferably dried in a warm atmosphere prior to projection. Such printed sheets of foil are quite permanent in character, due to the fact that our ink, although it keeps moist for a long time on the inking pad, can be

dried after printing by using warm air, making thereby a permanent record for projection purposes. There can therefore be produced by our invention, wide sheets of foil with characters

stamped thereon for conveying news, illustrations, cartoons and the like, for projection purposes.

As stated, the ordinary inks or marking fluids containing glycerine as the liquid vehicle do not produce satisfactory markings on cellulose acetate foil. Accordingly we have developed an ink for this purpose comprising a dye, pigment or lake, and a liquid solvent plasticizer for cellulose acetate or other organic derivative of cellulose. An example of such marking ink for cellulose acetate foil is:

| Parts by weight                                     |    |
|-----------------------------------------------------|----|
| Dye (such as Methyl Violet)                         | 18 |
| Triacetin                                           | 41 |
| Mixture of ortho- and para-ethyl toluene sulfonamid | 41 |

The dye is ground in the triacetin and ethyl toluene sulfonamid. Other suitable coloring materials may be used instead of the Methyl Violet. The triacetin and ethyl toluene sulfonamid may be replaced in whole or in part by other cellulose acetate plasticizers such as a dimethyl phthalate, dibutyl tartrate or mono-methyl xylene sulfonamid. We have also found that high boiling solvents such as glycol diacetate (b. p. 186° C.) or benzyl alcohol (b. p. 206° C.), in amounts of say 5 to 25 parts by weight, may be added to the above formula to regulate the rate of drying. The principle of the invention with respect to our ink is to employ an agent or liquid that exerts a solvent action on the cellulose acetate or other organic derivative of cellulose in the foil.

Our ink or marking fluid is superior to the ordinary glycerine ink not only when used for marking cellulose acetate foil but when used in connection with reconstituted cellulose foil or glazed paper, since it is not as hygroscopic as glycerine ink and is readily absorbed by glazed paper or reconstituted cellulose foil.

It is to be understood that the foregoing detailed description is given merely by way of illustration and that many variations may be made therein without departing from the spirit of our invention.

Having described our invention, what we desire to secure by Letters Patent is:

1. A printing ink adapted to be used for printing on transparent strips consisting of a coloring material dispersed in a liquid consisting of a non-hygroscopic solvent plasticizer for derivatives of cellulose selected from the group consisting of triacetin, ethyl toluene sulphonamides, dimethyl phthalate, dibutyl tartrate and mono-methyl xylene sulphonamide.

2. A marking fluid consisting of a dyestuff dispersed in a liquid consisting of triacetin and ethyl toluene sulfonamide.

3. A liquid ink consisting of a coloring agent dissolved in dibutyl tartrate substantially free from cellulose derivatives.

4. A liquid ink comprising a coloring agent dissolved in dibutyl tartrate substantially free from cellulose derivatives.

MILLARD DEMAREST.  
KIRTLAND FLYNN.